

Oct. 5, 1948.

J. W. BAYMILLER

2,450,408

TEXTILE FIBER DRAFTING ELEMENT

Filed Sept. 16, 1943

FIG. 1



FIG. 2



FIG. 3



Inventor  
John W. Baymiller  
by  
Walter & Kauffman  
Attorney

## UNITED STATES PATENT OFFICE

2,450,408

## TEXTILE FIBER DRAFTING ELEMENT

John W. Baymiller, Manheim Township, Lancaster County, Pa., assignor to Armstrong Cork Company, Lancaster, Pa., a corporation of Pennsylvania

Application September 16, 1943, Serial No. 502,553

6 Claims. (Cl. 19—131)

1

This application is a continuation-in-part of my copending application Serial No. 457,717, now abandoned, entitled "Textile fiber drafting elements and method of making the same," and filed September 9, 1942.

This invention relates to drafting aprons, spinning rolls, drawing rolls, and the like used in the textile industry and commonly known as textile fiber drafting elements. The invention finds particular usefulness in the so-called long draft aprons used in the drafting of fibers, particularly rayon, and in the spinning roll covers used in drawing fibers, such as cotton, rayon, and the like.

The invention will be described with particular reference to long draft spinning aprons but it is here pointed out that the invention is not limited to aprons. Additionally, the example chosen for illustration is used in the drafting of rayon fibers since the invention finds unusual commercial acceptability in that field. Here again, it is pointed out the invention is not limited to textile fiber drafting elements for the processing of rayon. It contemplates all textile fiber drafting elements, regardless of the particular work performed or the type of fibers operated upon.

The invention also includes a method of treating textile fiber drafting elements to improve their working surfaces.

In drafting rayon fibers in accordance with the Whitin-Casablancas long draft system and systems of a similar nature, the front and back rolls are the same as those used on a regular three-roll drafting frame. However, in place of a pair of middle rolls to engage the fiber under treatment, a pair of aprons is provided which reaches forward close to the nip of the front rolls. The back rolls and aprons serve to break draft the roving and the front rolls and aprons perform the main draft. The aprons support and control the loose fibers over a considerable portion of their length as they move from the back pair of rolls into the nip of the front pair of rolls. With this system, because of the better control of the fiber within the principal drafting zone, it is possible to use high drafts and produce uniform, strong yarn. In the Saco Lowell-Roth system a similar apron is used with an upper roll instead of a second apron.

The aprons heretofore have been made extensively of leather. Attempts have been made to utilize synthetic rubber aprons but acceptable operation of these has been limited largely to the processing of the shorter staple fibers. When

2

synthetic rubber aprons have been tried on longer staple fibers, such as rayon, it has been found that the frictional resistance or grip of the apron surface is so great that a positive "holding" action is exerted against the drafting of the front rolls resulting in broken fibers, a mutilated roving, and excessive waste which collects and falls into the roving, causing defective work. For these reasons, synthetic rubber aprons have been completely inoperative in many instances on long staple rayon. These results indicate that a similar action probably takes place in the processing of the shorter staple fibers such as cotton but to a lesser degree. Improved results in the processing of such fibers should be attained by my invention, although satisfactory operation is now obtained on such short staple fibers with the synthetic rubber aprons now available.

There has also been a noticeable tendency for the synthetic rubber aprons to be damaged or destroyed because of failure of the apron to move freely over the stationary supporting bar in the Whitin-Casablancas, the Saco Lowell-Roth, and other similar systems; the physical characteristics of the inner surface of the aprons impairing their movement over the stationary surface under usual drafting tension.

In drawing textile fibers, one commonly employed machine is the drawing frame which includes a series of spaced pairs of drawing rolls, the lower roll of each pair being in the form of a fluted metal roll. The upper roll of each pair in certain types of drawing frames has a resilient working surface and in many such units the upper rolls are covered with cork composition, leather, and synthetic rubber. Front rolls covered with these materials give considerable difficulty in operation due to the fact that fibers, particularly rayon fibers, tend to stick to the rolls and "lap up" on or wrap around the front roll. Synthetic rubber is especially susceptible to "lapping up." This fiber drawing illustration has been given as typical of the problems involved in fiber drafting. The same or similar difficulties may be encountered in roving frames, spinning frames, and in worsted and woolen processing equipment as well as in other services where fiber drafting elements are used.

From the foregoing it will be clear that the use of synthetic rubber surfaces in the drafting and spinning of textile fibers, particularly rayon and similar long staple fibers, has met with limited success. In the case of aprons used in long drafting, the frictional qualities of the synthetic rubber aprons have been too great, resulting in

breaking of the fiber and concomitant mutilated rovings, as well as damage or destruction of the aprons due to impaired movement of the aprons over the stationary supporting bars. In the case of drawing rolls, the problem has been one oflapping up on the front roll due to excessive affinity of the synthetic rubber for the fibers.

Synthetic rubbers are well suited in many respects for textile fiber drafting. They possess oil resistance, a major prerequisite of a fiber drafting element. They are extremely flexible, do not crack or materially change their shape upon continued flexing, nor do they alter their shape or physical characteristics to any material degree with changes in humidity. Leather, the material most commonly used for aprons up to the present time, is lacking in these qualities.

It is an object of my invention to provide a textile fiber drafting element possessing the foregoing desirable characteristics of synthetic rubbers and at the same time possessing an improved working surface which overcomes the difficulties heretofore encountered. Another object of my invention is to improve the inner synthetic rubber surface of drafting aprons to provide a surface which will permit unimpaired movement of the aprons under usual drafting tension. It is a further object of my invention to provide a method whereby these desired surface characteristics may be imparted to synthetic rubber textile fiber drafting elements.

The synthetic polymerization products of open-chain aliphatic conjugated dienes, particularly those having the formula  $H_2C=CR-CH=CH_2$ , wherein R is hydrogen, a halogen, or a methyl radical, are useful in the practice of my invention for they respond well to my treatment. The polymerization products of butadiene, chloroprene, and isoprene, such as polybutadiene, butadiene-acrylonitrile, butadiene-styrene, and butadiene-isobutylene copolymers; polychloroprene; polyisoprene; and isoprene-acrylonitrile copolymers, all have the formula  $H_2C=CR-CH=CH_2$ , wherein R is as defined above, and the polymerization products of this class of polymerizable open-chain aliphatic conjugated dienes is preferred.

In the course of experimental work in connection with the manufacture of textile fiber drafting elements, I have discovered that those vulcanized or unvulcanized synthetic polymerization products of open-chain aliphatic conjugated dienes which in their final form have a carbon to carbon bond may be treated with a free halogen, to thereby change the surface characteristics of the product. By such treatment, the surface characteristics of the product are materially altered, and improved; all affinity which would cause "lapping up" is eliminated; the frictional characteristics of the surface are changed, resulting in a surface ideally suited for the long drafting of rayon and other fibers heretofore difficult to work; and all tendency for aprons to be damaged or destroyed because of impaired movement over the stationary supporting bars is eliminated. Drawing rolls produced from such composition and having the treated surface have been found to work satisfactorily on rayon and long staple cotton, while untreated rolls of the same composition operating in an adjacent frame have lapped up to a degree sufficient to make their use impracticable. Likewise, long draft aprons formed from such composition and so treated have been found to operate remarkably well on machines employing the Whitin-Casa-

blancas long draft system without undue tearing or breaking the fibers, whereas untreated aprons operating in an adjacent frame have proved inoperative on rayon fibers.

I will describe a long drafting apron produced in accordance with my invention using a vulcanized butadiene-acrylonitrile composition as the base. A composition may be formed from the following constituents:

|                                   | Parts by weight |
|-----------------------------------|-----------------|
| Butadiene-acrylonitrile copolymer | 100             |
| Sulfur                            | 1.5             |
| Zinc oxide                        | 5               |
| Phenyl-beta-naphthylamine         | 1               |
| 15 Dibutyl phthalate              | 10              |
| Stearic acid                      | 1               |
| Semi-reinforcing carbon black     | 50              |
| Benzothiazyl disulfide            | 1.5             |

20 In the foregoing example, butadiene-acrylonitrile copolymer is the base composition, sulfur is the vulcanizing agent, zinc oxide is an activator, the phenyl-beta-naphthylamine is an anti-oxidant, the dibutyl phthalate is a plasticizer, the 25 stearic acid is also an activator and may be omitted, and the benzothiazyl disulfide is an accelerator.

As will be more fully discussed, other synthetic polymerization products may be substituted for 30 the butadiene-acrylonitrile copolymer and the product may be vulcanized or unvulcanized, depending upon the service to be performed. As is obvious, the base composition may be compounded with various ingredients to produce a final product having the desired physical properties.

This material is formed into an apron in the desired manner, with or without a backing cloth, fabric, or reinforcing cord. A preferred practice is to provide an inner layer of a polymerization

40 product of an open-chain aliphatic conjugated diene into which a reinforcing cord is embedded and to superimpose a layer of a polymerization product of an open-chain aliphatic conjugated diene thereover to constitute the outer portion.

45 The whole is then cured and vulcanized. After curing and vulcanization, the outer surface is buffed to the desired fineness. This apron is found to have an outer working surface which in itself would not be satisfactory for drafting long 50 staple rayon. The apron thus formed is subjected to the action of a free halogen for a period of time sufficient to permit a chemical reaction to take place at the desired surfaces of the apron. Preferably, with drafting aprons both the inner 55 and outer working surfaces are treated but either surface may be selectively treated if this is desired.

As a specific example, the apron may be immersed in a water solution of chlorine, the 60 strength of which is equivalent to 6 to 8 cc. of a tenth normal sodium thio-sulfate solution, for a period of about twenty minutes. The chlorine water may be prepared by passing chlorine gas into water until the required strength is obtained, 65 by acidifying a solution of a chlorine compound such as sodium or calcium hypochlorite, an organic solution of chlorine may be used, or any other means of getting free chlorine into contact with the surface of the polymerization product.

70 The strength of the chlorine solution is not critical provided, of course, there is free chlorine present. The desired chemical reaction will take place in a very weak solution or in a substantially saturated solution. The duration of the treatment is not critical but depends upon the halogen

used, the degree of unsaturation of the polymerization product, the strength of the treating solution and other variable factors.

After the twenty-minute immersion in the chlorine water, the apron is removed and dried. If solutions of sodium or calcium hypochlorite have been used, it is advisable to wash the aprons after treating in order to remove any trace of deposited salts.

In place of chlorine, any other halogen may be used, such as fluorine, bromine or iodine. Fluorine is so chemically reactive that its use is commercially impracticable and bromine and iodine are not as reactive as chlorine. Therefore, I prefer to use chlorine because it is cheap, readily available, clean, light-colored, and sufficiently active to produce satisfactory results in a relatively short period of time.

The polymer unit of the butadiene-acrylonitrile composition referred to in the foregoing example has the following formula:



I believe that upon treatment with a halogen, the carbon to carbon double bond in the polymer is saturated and the material at the surface which has been treated would have the following formula:



It is recognized that vulcanization causes a modification of the polymer but I have found that the final effect of the halogen treatment is substantially the same when applied to the polymerization product in either the vulcanized or unvulcanized state.

Other polymerization products which have the following chemical polymer formulas may be treated in accordance with this invention:



Polybutadiene



Butadiene-styrene



Butadiene-isobutylene



Polychloroprene



Polyisoprene



Isoprene-acrylonitrile

It will be observed that in each of the foregoing examples there is a degree of unsaturation represented by the carbon to carbon double bond and any synthetic polymerization product of an open-chain aliphatic conjugated diene in which there is a substantial degree of unsaturation, represented by carbon to carbon double bonds in the polymerization product will be found to work satisfactorily. Of course, those polymerization products having a high degree of unsaturation will be more reactive than those of a lesser degree

of unsaturation. Where the degree of unsaturation is low, it is desirable for best results to increase the proportion of the conjugated diene in the copolymer.

In addition to the attack at the carbon to carbon double bond which is believed to constitute the major part of the reaction, there may also be some substitution of halogen for hydrogen but, in any event, the final result is the production of a product having an improved surface for textile fiber drafting. It should be remembered that the foregoing polymer formulas each represent a single polymer unit and highly polymerized products having a high molecular weight with an unsaturated bond in the polymer units will possess a high degree of unsaturation sufficient even after vulcanization to the desired degree to be highly receptive to the halogenation treatment.

It will be understood that this is purely a surface treatment and that the reaction does not take place throughout the entire thickness of the apron. If the fiber drafting unit is rebuffed after use, because of wear, it will be necessary to retreat it in order to again provide the desired surface.

I have established that the reaction which takes place and provides the desired working surface is not an oxidation reaction which might be expected in the treatment of such organic materials with halogen and water. I have treated butadiene-acrylonitrile copolymers and other polymerization products having a high degree of unsaturation with hydrogen peroxide in ammonium hydroxide thereby liberating oxygen very rapidly and have found no substantial difference in the surface characteristics of the products so treated. On the other hand, I have treated the same materials with an organic solution of chlorine such as an ethylene dichloride solution of chlorine thus eliminating all oxygen and have obtained the same results as when the materials were treated with a chlorine water solution. This establishes that the reaction is not an oxidation reaction but a halogenation reaction.

I have treated polymerization products which do not have the carbon to carbon double bond and have found that no substantial change in the surface characteristics occurs. For example, I have treated the material known as "Koroseal" and having a polymer formula as follows:



The surface was not changed. Apparently, the reaction takes place only with those polymerization products having carbon to carbon double bonds or at least the reaction is sufficiently great to be important only in such compositions.

In the attached drawing:

Figure 1 is a diagrammatic view illustrating a so-called long draft apron as employed in the Saco Lowell-Roth system;

Figure 2 is a similar view showing the Whitin-Casablanca system; and

Figure 3 is a perspective view showing an apron having inner and outer working surfaces treated in accordance with my invention.

In both the Saco Lowell-Roth and Whitin-Casablanca systems as illustrated, the drafting aprons move over a stationary supporting bar. This bar is indicated at 2 in Figure 1 and at 3 in Figure 2. The apron 4 in Figure 1 is driven by a roll 5 and a tension roll 6 and guide roll 7 are provided. The roving 8 is drafted between the pair of back rolls 9, front rolls 10, and intermediate roll 11. The fiber is supported during draft-

ing by the apron 4 moving over the stationary supporting bar 2 and the driving roll 5, drafting tension being supplied to the apron by the tension roll 6.

In the Whitin-Casablanca system shown in Figure 2, the drafting is accomplished between the pair of back rolls 12 and front rolls 13. In this system a pair of drafting aprons 14 and 15 is provided, the lower apron 15 is driven by roll 16 and the upper apron is driven by frictional engagement with the lower driven apron. A guide roll 17 is provided and this roll is weighted to obtain the desired pressure between the aprons. The roving 18 is supported and operated upon by the aprons moving over their stationary supporting bars 3 and rolls 16 and 17.

Figure 3 illustrates a typical drafting apron embodying my invention. It consists of an outer portion 18 of a synthetic polymerization product of an open-chain aliphatic conjugated diene such as the butadiene-acrylonitrile copolymer of the example previously referred to and an inner portion 19 formed of the same composition and preferably having a helically disposed reinforcing cord embedded therein. In this embodiment, both the inner and outer working surfaces are indicated as having been treated. Of course, with cots and other drafting elements where there is no problem of impaired movement only the outer working surface may be treated and in drafting aprons it may be desirable to treat but one of the surfaces, although the simplicity of the process where the article is immersed in the treating solution recommends itself for most articles.

For most textile drafting purposes oil resistance is desirable in the drafting element and, where this is a factor, the oil resistant polymerization products, such as the copolymers of butadiene and acrylonitrile, isoprene and acrylonitrile, and polymerized chloroprene will be generally preferred.

While I have illustrated and described certain preferred embodiments of my invention, it will be understood that the same may be otherwise embodied and practiced within the scope of the following claims.

I claim:

1. A lap-resistant textile fiber drafting element having a fiber working surface comprising the reaction product of a free halogen and a vulcanized synthetic polymerization product of an open-chain aliphatic conjugated diene, said polymerization product having carbon to carbon double bonds, said fiber working surface being characterized by its lap resistance.

2. A lap-resistant textile fiber drafting element having a fiber working surface comprising the reaction product of free chlorine and a vulcanized synthetic polymerization product of an open-chain aliphatic conjugated diene, said polymerization product having carbon to carbon double bonds, said fiber working surface being characterized by its lap resistance.

3. A lap-resistant textile fiber drafting element having a fiber working surface comprising the reaction product of a free halogen and a vulcanized copolymer of butadiene and acrylonitrile, said fiber working surface being characterized by its lap resistance.

15 4. A lap-resistant textile fiber drafting element having a fiber working surface comprising the reaction product of free chlorine and a vulcanized copolymer of butadiene and acrylonitrile, said fiber working surface being characterized by its lap resistance.

20 5. A lap-resistant textile fiber drafting element having a fiber working surface comprising the reaction product of a free halogen and a copolymer of isoprene and acrylonitrile, said copolymer containing carbon to carbon double bonds and having a substantial degree of unsaturation, said fiber working surface being characterized by its lap resistance.

25 6. A lap-resistant textile fiber drafting element having a fiber working surface comprising the reaction product of a free halogen and a vulcanized polymerization product of chloroprene, said fiber working surface being characterized by its lap resistance.

30 35 JOHN W. BAYMILLER.

#### REFERENCES CITED

The following references are of record in the file of this patent:

#### UNITED STATES PATENTS

| Number    | Name     | Date          |
|-----------|----------|---------------|
| 1,532,234 | Dennison | Apr. 7, 1925  |
| 1,810,560 | Garvey   | June 16, 1931 |
| 2,012,223 | Cutler   | Aug. 20, 1935 |
| 2,126,733 | Catt     | Aug. 16, 1938 |
| 2,132,268 | Mallard  | Oct. 4, 1938  |
| 2,201,931 | Sullivan | May 21, 1940  |
| 2,287,780 | Carman   | June 30, 1942 |
| 2,293,266 | Mitchell | Aug. 18, 1942 |
| 2,304,656 | Rockoff  | Dec. 8, 1942  |
| 2,341,656 | Rockoff  | Feb. 15, 1944 |